

Jan. 28, 1936.

J. J. POHLMANN

2,028,948

DECORATIVE PAPER AND METHOD OF MAKING THE SAME

Filed Nov. 7, 1934

*FIG. 1.*



*FIG. 2.*



*FIG. 3.*



*FIG. 4.*



*FIG. 5.*



INVENTOR  
JOSEPH J. POHLMANN  
BY  
*Clapin & Neal*  
ATTORNEYS

## UNITED STATES PATENT OFFICE

2,028,948

DECORATIVE PAPER AND METHOD OF  
MAKING THE SAME

Joseph J. Pohlmann, South Hadley Center, Mass.,  
assignor to The Beveridge-Maryellum Company, Holyoke, Mass., a corporation of Massachusetts

Application November 7, 1934, Serial No. 751,879

2 Claims. (Cl. 41—26)

This invention relates to the decoration of paper, and more particularly to an improved method of the type in which a crystallizable material in a lacquer containing volatile solvent is applied to the paper and such material permitted to form a crystalline pattern upon evaporation of the solvent. According to the prior practices of producing crystalline coated papers, the characteristic appearance has resided solely in the crystalline formation and the contrast afforded by the mat and glossy areas resulting from growth of the crystals on the surface of the paper. It is the object of my invention to provide a method of decorating paper and employing the steps of forming a crystalline structure over the surface of the paper which will give to the crystals so formed an appearance of iridescence or opalescence and depth not obtainable from the crystal coating alone.

20 In the accompanying drawing, which diagrammatically illustrates certain of the steps of the method of this invention,

Fig. 1 shows in diagrammatic form the appearance of the finished paper;

25 Fig. 2 shows diagrammatically the first step of the method;

Fig. 3 shows diagrammatically the second step;

Fig. 4 is a similar view showing the third step;

30 Fig. 5 is a diagrammatic view on a greatly enlarged scale showing features of the first step comparable with the showing of Fig. 2; and

Fig. 6 is a view similar to Fig. 5 but comparable with the showing of Fig. 3.

As the first step of the method, the paper 9 is passed through a printing operation to apply color in irregularly shaped areas as shown in Fig. 2 at 10. The color in these areas is applied in the form of dots as indicated at 11 in Fig. 5, the dots being variously spaced as shown in the latter figure so that the intensity of the color varies over the irregular areas as will be obvious from the grouping of the dots in Fig. 5. While for the purpose of illustration the color areas are shown of uniform intensity and with clearly defined edges in Fig. 2, it will be obvious from Fig. 5 that in actual practice there is no clearly defined boundary especially where the color intensity is very light. For purposes of illustration the first color application is shown as orange which should be relatively light in shade. The sheet to which the first color has been applied is now run through the press a second time. The printing surface used may be the same as for the previous printing but out of register with the first so that the succeeding color areas overlap

the others con-conformably. It is not necessary to attempt any particular relation with reference to the degree of off registration between the two printings. In practice the sheet is merely run through the press hit-or-miss and since it would be practically impossible to secure exact registration even if desired a satisfactory degree of non-conformity is invariably obtained. The application of the second printing is diagrammatically shown in Fig. 3 at 12, the color blue being indicated. The "gross" effect of the combined printings is indicated in Fig. 3 where certain color areas overlap as at 13 resulting in a compound color. Other areas show the single colors with interspersed areas of white. Due to the application of colors in variously spaced dots a further variety of effect is obtained as indicated in Fig. 6, where the dots of the second color are indicated in dotted line as at 14. For example, inasmuch as in some places (1) a maximum intensity of blue falls on the areas of maximum intensity of the orange; (2) a maximum intensity of blue falls on a minimum intensity of orange; (3) a minimum intensity of blue falls on a maximum intensity of orange; (4) a minimum intensity of blue falls on a minimum intensity of orange. There are of course similar combinations of intermediate intensities as well as areas covered by varying intensities of a single color.

30 The sheet is then once more passed through the press and a third color indicated as pink at 15 is applied as before out of register with the two preceding colors. The result is diagrammatically indicated in Fig. 4 and it will be appreciated that there is thereby obtained various combinations and permutations of the three colors and their various intensities along the lines indicated above.

As previously stated, the drawing is purely diagrammatic. In practice the color areas, far from having the clear cut definition indicated by the figures of the drawing in which conventional cross-hatching is used to indicate color, give an almost indefinable cloudy appearance. Moreover, the shades used are preferably so light that a single printing is more suggestive of color than productive of a definite colored appearance. With the addition of each successive color the degree of color sensation is increased, mainly as the result of the appearance of those areas where the maximum intensity of the several colors have been superposed. The shades produced by the combination of two or more colors are widely and irregularly scattered and variable as to hue and

intensity, and the general effect is a softly mottled cloudy appearance, the arrangement and relation of the colored dots being apparent only from a microscopic examination.

- 5 Over the paper thus prepared a crystallizing solution is spread in any usual or preferred manner and permitted to crystallize as is diagrammatically indicated at 16 in Fig. 1. The effect produced by the colored areas as they appear 10 through the crystalline structure is to give to the crystals an effect of iridescence which is the result not only of the colors themselves but of the varying texture of the crystals which modify the color effects. This iridescence is diagrammatically suggested in Fig. 1 by the varying 15 areas of surface shading 17 and stippling 18. If desired the crystalline solution may be tinted to supply part of the iridescent effect or to modify and vary the effect of the underlying colors as 20 a whole. For example by using a grey tinted crystalline solution a mother-of-pearl effect may be obtained whereas cream or pink tinted solutions produce respectively yellow or pink pearl effects.
- 25 While the color areas are above described as applied by successive off register printings, it will be understood that the color areas may be supplied by spraying or other ways by which the desired non-conformity of the areas is obtained.
- 30 The color may be applied while the paper is still on the paper machine and the varying in-

tensities secured by the varying absorption of the color by the moist paper, or the finished paper can be moistened.

It will be understood that the invention is not limited to the specific colors above mentioned and that the colors will be chosen in view of the exact effect desired.

I claim:

1. The method of decorating paper which comprises successively and non-conformably applying to the surface of the paper a plurality of irregular areas of at least two colors, said areas having no defined boundaries and being formed of dots of color, light in shade, and variously spaced to provide various color intensities over the several areas, and thereafter forming thereon an unbroken translucent crystalline coating.

2. A decorated paper comprising a paper sheet having irregular areas respectively of orange, blue and pink color, said areas being formed of small dots of color varying in spacing, the colors being light in shade and the several color areas non-conformably overlying each other, and an unbroken translucent crystalline coating overlying the colors, the color combinations and permutations produced by the non-conforming color areas appearing through the facets of the crystals with a characteristic appearance of cloud-like iridescence.

JOSEPH J. POHLMANN. 30